

Patented July 28, 1925.

1,547,445

# UNITED STATES PATENT OFFICE.

GEORG REINHART, OF MUNICH, GERMANY, ASSIGNOR TO REINHARTEN-WERK  
CHEMISCHE FABRIK GES. M. B. H., OF MUNICH, GERMANY.

## NONCORROSIVE COOLING AGENT.

No Drawing.

Application filed May 8, 1922. Serial No. 559,412.

*To all whom it may concern:*

Be it known that I, GEORG REINHART, a citizen of the German Republic, residing at Munich, Germany, have invented certain 5 new and useful Improvements in Noncorrosive Cooling Agents, of which the following is a specification.

The present invention relates to improvements in the provision and use of liquid 10 cooling and refrigerating agents of low freezing point, with the object of forestalling freezing thereof and particularly of preventing corrosion thereby of the metallic structural elements used in the construction 15 of the refrigerator or other container.

The main drawback attaching to the use 20 of the well known liquid cooling media or freezing mixtures is that they all more or less are apt to corrodingly attack the metal container material, and to bring this about it suffices that a metal, a metal alloy, or a 25 soldering agent is used in the construction of the refrigerator structure the normal potential of which is more negative than that of the calcium (Ca) or magnesium (Mg) of the best known refrigerant.

Thus, for instance, barium, whose normal 30 potential equals minus 3, 1 presents a more negative normal potential than cadmium with its normal potential of minus 2, 8; and, further, barium has a more negative normal potential than magnesium of minus 1.83.

To a structural element of barium metal 35 then there never would be imparted a deposit of magnesium or calcium, since the metal element itself would be dissolved for the reason that the dissolving tension of this more negative metal is greater than 40 that of the Mg or Ca respectively, with the result that the barium refrigerator parts would be corroded.

This corrosive action is effectively obviated 45 if the cooling solution is composed of metal salts which on the one hand differ to some extent from one another in normal potential, and on the other hand show a more pronounced negative normal potential than the metal used in the construction of 50 the refrigerator or other container, or if there are several metals or alloys, than the most negative of such metals used. In this instance, if at any point in the refrigerator even only a trace of the solution metal is 55 deposited, there will be a deposit on the

most negative metal, the point of deposit serving as anode. It is these deposits, and not the refrigerator metals, between which the local action, that is the electrical dissolving process, is initiated and carried on. 60 A corrosion of the refrigerator metal is thus effectively prevented.

By way of example: The practical experiments with light metals, for instance magnesium and calcium have already progressed so far that magnesium alloys can now successfully be used in the manufacture of refrigerators. To guard against corrosion of the Mg alloy structural parts I propose to employ in place of the magnesium-calcium chloride solution ( $MgCl_2 - CaCl_2$ ) a  $CaCl_2$  solution to which has been added a small amount of potassium chloride (KCl). The concentration of this solution is dependent upon the lowest operative temperature. 70

Zinc will be found in the solder of every modern metal refrigerator, for which reason for practical purposes only such metal salts enter into the present solution the metals 80 of which show a more negative normal potential than zinc, as for instance the salts of magnesium (-1.83), of calcium (-2.8), of sodium (-2.99), of barium (-3.1) and of potassium (-3.2). Expressly excluded are the salts which contain, beside one of the stated metals, a further metal of more positive normal potential; thus for instance chromic compounds of potassium or sodium cannot be used since they contain, beside the potassium (-3.2) or the sodium (-2.99), chromium with a normal potential of -0.8, and as such for our purposes too high. 90

If a chromic compound of potassium or sodium were used, the electrolyte would contain a metal ion whose normal potential is more positive than the normal potential of the zinc used in the refrigerator material, with the result that the latter would then be corroded. 95

For best results the normal potentials of the two salts should not differ very materially.

What I claim is:—

1. Non-corrosive cooling agent of low freezing point, consisting of an aqueous solution of magnesium chloride and calcium chloride. 103
2. Non-corrosive cooling agent of low freezing point, consisting of an aqueous so- 116

lution of substantially 80% magnesium chloride and substantially 20% calcium chloride, the solution having a density of approximately 25° Bé.

5 3. Non-corrosive cooling agent of low freezing point, consisting of an aqueous solution of magnesium chloride and calcium chloride, the former in predominant

amount, and a relatively small percentage of potassium chloride.

In testimony whereof I affix my signature in presence of two witnesses.

GEORG REINHART.

Witnesses:

ALBERT HALSTENER,  
ALEXANDER DE SOTO.